

March 14, 1944.

G. CROMPTON, JR

2,343,957

PERIPHERAL DIAMOND ABRASIVE WHEEL AND METHOD OF MAKING SAME

Filed April 2, 1942



Fig. 3 Fig. 4 Fig. 5 Fig. 6

Fig. 2



FIG. 1

Inventor

George Jacob Frank.

## UNITED STATES PATENT OFFICE

2,343,957

PERIPHERAL DIAMOND ABRASIVE WHEEL  
AND METHOD OF MAKING SAMEGeorge Crompton, Jr., Worcester, Mass., assignor  
to Norton Company, Worcester, Mass., a corporation of Massachusetts

Application April 2, 1942, Serial No. 437,374

5 Claims. (Cl. 51—309)

The invention relates to peripheral diamond abrasive wheels and methods of making them, and with regard to its more specific features to wheels having a single layer of diamonds.

One object of the invention is to provide an inexpensive peripheral diamond wheel. Another object of the invention is to provide a single layer diamond abrasive wheel of relatively long life. Another object of the invention is to provide a practical commercial method for making wheels of the class indicated which will permit the ready duplication of results.

Another object of the invention is to orient and distribute the diamonds or other abrasive grains on the peripheral surface of a backing, whereby a uniform and efficient grinding action will be secured. Another object of the invention is to provide an efficient apparatus and method for the electrostatic deposition of diamond abrasive upon a circular backing. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein, and the scope of the application of which will be indicated in the following claims.

In the accompanying drawing illustrating one of many possible embodiments of the mechanical features of the invention,

Figure 1 is a vertical sectional view of apparatus for making the wheel according to the invention, some of the parts being shown in elevation;

Figure 2 is a view, on an enlarged scale, of a portion of the wheel backing showing the application first of a coating of solder and then of diamonds;

Figure 3 is a fragmentary radial sectional view of the backing showing the periphery;

Figure 4 is a view similar to Figure 3 showing a layer of solder;

Figure 5 is a view similar to Figure 4 showing a layer of diamonds in the solder;

Figure 6 is a view similar to Figure 5 showing an additional layer of metal which has been applied, for example, by an electroplating process.

Referring first to Figure 1, I provide a hopper 10 containing diamonds 11 and having a cover plate 12 to keep out dust. A hole 13 admits air to prevent the formation of a vacuum. The hopper has at the lower part thereof approaching walls 14 and 15 and the wall 14 contacts a roller 16.

The wall 15 is just clear of the roller 16 and a slidable gate 17 can be adjusted to more or less clearance from the roller 16. The roller 16 is on a shaft 18 which is fastened to a pulley 19 over which runs a belt 20 driven from any suitable source of power, not shown. The pulley 19 is driven clockwise, thus driving the roller 16 clockwise to discharge diamonds under the gate 17. This produces a waterfall of diamonds descending from the right-hand side of the roller 16. The gate 17 could be on the other side and the roller 16 could move counterclockwise to discharge the waterfall on the left-hand side of the roller 16.

A suitable source of power, not shown, drives a belt 21 around a pulley 22 on a shaft 23 to which is fastened a roller 24 which is thus rotated, in this case in a counterclockwise direction. Around the roller 24 passes a belt 25 which also passes around idler rollers 26 and 27. The width of the belt 25 is substantially the same as that of the roller 16 and the belt 25 picks up the waterfall of diamonds and moves them to the left. Any suitable tray, not shown, may be placed under the belt to catch diamonds that bounce off the belt or fall off at the edges. The roller 27 is grounded.

Another belt 30 driven from a suitable source of power, not shown, passes around and rotates a pulley 31 which is fastened to a stud shaft 32 upon which is a nut 33 removably securing in place a wheel back 34. This wheel back is made of a suitable metal, for example, of German silver. The wheel back 34 is likewise shown in the remaining figures. It should be more or less of a disk having a peripheral surface 35 which is more or less of a cylinder. The width of the surface 35 should be substantially that of the width of the belt 25. The surface 35, however, may be a cone or may be undulating.

The shaft 32 is supported at the top of a frame 40 upstanding from a base 41. In any appropriate manner the shaft 32, nut 33, and wheel 34 are insulated. The frame 40 may be of metal and the parts mentioned may be insulated by an insulating bearing or else all or a portion of a frame 40 may be built of insulating material. It is preferred to place the whole structure upon an insulating plate 42.

Upstanding from the base 41 is a forked bracket 45 supporting a pin 46 which pivots a foot treadle 47 having an insulating tread 48. The other end of the treadle 47 is a fork 49 having pins 50 projecting into a groove 51 on the outside of a long vertical sleeve 52 which slides up and down on a shaft 53 but cannot turn thereon account

of a key 64. The shaft 63 is screwed into a plate 55 resting on and suitably fastened to the base 41. At the upper end of the sleeve 52 is a wheel 56 having an inwardly extending flange 57 engaging an outwardly extending flange 58 formed on the sleeve 52. On top of the sleeve 52 rests a hub 60 of the wheel 56 which is internally screw threaded and engages a screw shaft 61 which is non-rotatively guided in the sleeve 52 by means of a key 62. The hand wheel 56 has an insulating outer portion 63 by which it may be turned.

To the upper end of the shaft 61 by means of a nut 65 is fastened a box 66 having openings 67 on the under side and containing a burner pipe 68 upstanding from which are a plurality of burners 69. The pipe 68 is connected by means of a rubber hose 70 with a valve, not shown, and a source of gas. The rubber hose 70 serves at once as a flexible connection and another insulator.

The burners 69 extend through a hole 71 in the top of the box 66 and into a second box 72 which has a bottom opening 73 matching the opening 71. The box 72 contains refractory bricks 75 which are shaped to support the edges of a melting pot 76 and act both as heat insulators and electric insulators. The melting pot 76 is filled with suitable metal or solder, for example, hard German silver solder, copper 35; zinc 56.5; nickel 9.5.

In any suitable manner, that is, by the use of a bus bar and a high tension electric generating apparatus, electromotive force of high potential is maintained on the disk 34. This is diagrammatically indicated by a line 80. It was already noted that the roller 27 was grounded. The belt 25 is a dielectric material. The roller 27 might be energized by means of the line 81 or either of the lines 80 or 81 might be connected to ground. A uni-directional field, that is, derived from a constant source of voltage, is preferably maintained but under certain conditions alternating or pulsating current might be used. The exact electromotive force used will depend upon many circumstances but for the conditions I have in mind 10,000 volts may be used.

Preferably the apparatus includes a cooling device, such as a pair of nozzles 85 on the ends of pipes 86 having valves 87 to blow cold air on the sides of the disk 34. Preferably the air should not impinge the periphery of the disk but should impinge the sides near the periphery at an acute angle to the planes of the sides of the disks.

The operation of the apparatus is as follows: The peripheral surface 35 of the disk 34 may first be coated with a flux. Calcined borax is a good flux for hard solder. One effective way to add the flux is to sandblast the surface 35 until it is quite rough, then rub dried borax upon the surface.

The disk 34 is now mounted upon the spindle 32. The hard solder, such as that already mentioned, is then introduced into the melting pot 76 and the gas burners 69 are lighted. After a little time the solder melts. Then the belts 20, 21 and 30 are started and the operator steps upon the tread 48 of the treadle 47, raising the melted solder in the pot 76 into contact with the periphery of the disk 34. As soon as a film of liquid comes opposite the belt 25, the main switch, not shown, is closed creating the electrostatic field mentioned and at the same time the valve 87 is turned to apply the air blasts. Diamonds

jump from the belt 25 onto the surface 35 which is coated with a film of liquid 90. The diamonds 91 are evenly distributed and oriented in the liquid 90, as shown in Figure 5. The viscosity of the solder is high and the surface tension is great and so the diamonds do not fall out and shortly after they have contacted the liquid 90 the solder is congealed by the air blasts. When the advance end of the diamond coating just about reaches the liquid solder in the melting pot 76, the operator removes his foot from the tread 48 and lowers the pot 76. The coating operation, however, continues due to the already molten solder on the periphery 35. At this point 15 the air blasts from the nozzles 85 should be cut off to prevent premature solidification of the solder.

The hand wheel 56 with the insulating rim 63 is provided for adjusting the level of the liquid 20 from time to time. If desired a weight 95 connected to the sleeve 52 by a cord 96 going over a pulley 97 may be provided to balance part of the weight of the apparatus to prevent the operator from being fatigued in running this 25 apparatus.

After the wheel 34 is coated, as shown in Figure 5, it is desirable to apply a further layer, such as the layer 100 (Figure 6), of a tough metal to hold the diamonds 91 more firmly in position. 30 A suitable metal, such as nickel, may be applied in an electroplating bath which need not be described herein, since the electroplating of nickel is known. The sides of the disk 34 can be stopped-off during the electroplating operation.

Although a specific flux, a specific solder, a specific electroplating metal, and a specific metal for the disk 34 have been mentioned, it should be understood that other metals and combinations of metals and other fluxes may be used. 35 The object is to anchor the diamonds 91 securely to the disk 34. How much metal is used will depend upon how free-cutting the wheel is to be or whether, on the other hand, it should be highly resistant to wear and have a long life.

40 By causing the diamonds 91 to impinge upon the periphery of the disk 34 by means of an electrostatic field, they are evenly spaced and well distributed upon the periphery and at the same time well oriented to provide good cutting 45 edges and make a free-cutting grinding wheel. Lumping or crowding of abrasive in one spot is avoided, as also are thin places.

It will thus be seen that there has been provided by this invention a method, apparatus and an article in which the various objects hereinabove set forth together with many thoroughly practical advantages are successfully achieved. As various possible embodiments might be made of the mechanical features of the above invention and as the art herein described might be varied in various parts, all without departing from the scope of the invention, it is to be understood that all matter hereinbefore set forth or shown in the accompanying drawing is to be 50 interpreted as illustrative and not in a limiting sense.

I claim:

1. Method of making a grinding wheel comprising rotating a metal blank in a bath of molten metal while moving a supply of abrasive material in a continuous stream towards a surface of said metal blank which has a liquid film of metal from the metal bath, and transferring the abrasive from the stream to the metal blank by electrostatic attraction.

2. Method of making a grinding wheel comprising rotating a metal disk with its periphery in a molten metal bath, supplying abrasive to a conveyor which moves to a point adjacent the periphery of the metal blank, and forming an electrostatic field between the point and the periphery.

3. Method of making a grinding wheel comprising rotating a metal blank in a bath of molten metal while moving a supply of abrasive grains in a continuous stream to the surface of said metal blank which has a liquid film of metal from the molten bath, and thereafter metal plating an additional layer of metal around the abrasive grains by an electroplating operation.

4. Method of making a grinding wheel comprising rotating a metal blank with its periphery in a bath of molten metal, feeding abrasive grains

in a continuous stream to a point adjacent the periphery, and causing the abrasive grains to jump to the periphery by an electrostatic field.

5. A grinding wheel comprising a metal blank, a layer of relatively low melting point metal on a surface of said blank, diamonds evenly distributed and oriented with their greatest dimensions radial to the blank embedded in the relatively low melting point metal and constrictingly engaged by said low melting point metal by intimate contact of said low melting point metal entirely around the periphery of the embedded portions of said diamonds, and a further layer of relatively high melting point metal upon the layer of low melting point metal and surrounding the diamonds.

GEORGE CROMPTON, Jr.